

## UNITED STATES PATENT OFFICE

1,965,508

## METHOD OF TREATING WOOD FOR PROTECTING THE SAME FROM BLUING

John Tobias Olsson, Bollnäs, Sweden, assignor to  
 Stockholm Superfosfat Fabriks Aktiebolag,  
 Stockholm, Sweden, a corporation of Sweden

No Drawing. Application November 9, 1931,  
 Serial No. 574,844. In Sweden September 16,  
 1931

2 Claims. (Cl. 99—12)

The surfaces of sawn wood, especially at hot and damp weather, become blue-coloured during the drying of the wood which is caused by a number of microorganisms which rapidly grow on the surfaces of the wood as long as the temperature and the degree of moisture in the wood are favourable therefor. On account of the blue spots appearing on the surfaces of the wood the quality of the latter and also its value and usefulness for several purposes are reduced. The bluing or "blue surface" appearing yearly on sawn wood consequently means a national economic loss which is especially severe in case of wood to be exported.

15 The microorganisms causing the bluing are generally spread as spores, which stick to the surfaces of the wood where they, as long as the temperature and degree of moisture are favourable, develop themselves and grow rapidly. During 20 the continuous drying of freshsawn wood its content of moisture will gradually be lower than that which is necessary for the development of said microorganisms. Therefore, by applying antiseptic substances to the surfaces of the wood 25 it will be possible to prevent such development during the period required for decreasing the content of moisture of the wood to such a limit below which the development of said microorganisms cannot take place. Several antiseptic 30 substances have been proposed and used in practice for said purpose. It has for instance been proposed to treat the wood with a mixture of manganese salts of cresol sulphonic acids and chlorophenols. Each of these groups of substances has a powerful antiseptic action. The 35 reason for using a mixture of two or several antiseptic substances is this that the microorganisms in question belong to several species with different sensitivities. By using a mixture of two or several antiseptic substances there are, therefore, greater chances of preventing the development of the microorganisms in question, than if a single substance would be used for said purpose.

40 The use of manganese salts has, however, also the drawback that the wood surfaces after having dried become coloured brown. This colouring is no doubt feeble but anyhow distinctly visible. Moreover, said substances are somewhat irritating for the skin which is disagreeable for the workmen who are occupied with the treatment.

The present invention has for its object a method for preventing the bluing viz. the formation of "blue surfaces" on the wood which offers

the advantages that said drawbacks are removed and that the agent used is two or three times as efficacious as the above mentioned agent previously proposed. The present method consists in this that the new-sawn wood is dipped or submerged into an aqueous solution containing soluble salts or boron and chlorophenols, or that such solution is sprayed onto the surfaces of the wood or applied thereon in any other way. Investigations have proved that the soluble alkali salts of boron, for instance the sodium salt of tetraboric acid (borax), the sodium salt of metaboric acid and others have a very good capacity of preventing the development on the surfaces of wood of "bluing microorganisms" and that this capacity 60 can be utilized by applying a solution of said salts of the boric acid to the surfaces of the wood, for instance by dipping the wood into a solution of said salts. The action of said salts of the boric acid is, however, considerably increased if the 65 solution also contains chlorophenols, preferably chloro-meta-cresol. The simultaneous action of said substances has been found to be more efficacious than the action of each substance used separately in a corresponding quantity. It is 70 therefore sufficient that the solution is in contact with the wood surfaces for a relatively short time.

The pure chlorophenols are rather sparingly soluble in water. By the addition of alkali salts of the boric acid the solubility of the chlorophenols is considerably increased due to the formation of complex salts when the two constituents are at the same time dissolved in water.

This combination of two substances each of which has an antiseptic action, has for its object 85 to execute a more universal action on the different species of the microorganisms causing "blue surface" on the wood, and whose individual resistance is different. Due to the efficacious preservative action obtained by an aqueous solution 90 containing salts of boric acid as well as chlorophenols the solution may be used in a highly diluted state and has no irritating action on the 95 skin of the workmen and finally it does not at all colour the surface of the treated wood.

I claim:

1. The method of treating wood for protecting the same from bluing, consisting in exposing the surfaces of freshsawn wood to the action of an aqueous solution containing borax and chloro- 100 meta-cresol.

2. An agent for protecting wood from bluing, consisting of an aqueous solution of borax and chloro-meta-cresol.

JOHN TOBIAS OLSSON. 110